# EUROPEAN PATENT SPECIFICATION

(11) **EP 1 915 481 B1**
(45) Date of publication and mention of the grant of the patent: **26.09.2012**
(21) Application number: 06776618.8
(22) Date of filing: 04.08.2006
(51) Int. Cl.: D06M 10/02, D06P 5/20, D06P 3/24

(54) **PROCESS FOR PRINTING AND FINISHING ON FABRICS PARTIALLY OR TOTALLY CONTAINING ARAMIDIC FIBRE, IN THE FORM OF FILAMENT AND/OR FLOCK**
VERFAHREN ZUM BEDRUCKEN UND VEREDELN VON WENIGSTENS ZUM TEIL ARAMIDFASER IN FILAMENT- UND/ODER FLOCKENFORM ENTHALTENDEN TEXTILEN FLÄCHENGEBILDEN
PROCEDE D'IMPRESSION ET DE FINITION DE TISSUS ETANT CONSTITUES EN PARTIE OU EN TOTALITE DE FIBRES ARAMIDES, SOUS FORME DE FILAMENTS ET/OU DE FLOCS

(30) Priority: 12.08.2005 IT MI20051577
(43) Date of publication of application: 30.04.2008
(73) Proprietor: Mascioni S.p.A., 21030 Cuvio VA (IT)
(72) Inventor: CANONICO, Paolo, I-21052 Busto Arsizio (Varese) (IT); FASANA, Egidio, I-22100 Como (IT)
(74) Representative: Rapisardi, Mariacristina
(86) International application number: PCT/EP2006/007747
(87) International publication number: WO 2007/019977

(56) References cited:
- EP-A- 0 191 680
- EP-A2- 0 492 649
- WO-A1-00/10703
- GB-A- 2 053 026
- US-A- 5 622 773
- DATABASE WPI Week 198745 Derwent Publications Ltd., London, GB; AN 1987-316608 XP002409200 & JP 62 223384 A (ASAHI CHEM IND CO LTD) 1 October 1987 (1987-10-01)

## Description

The present invention refers to a new process for printing and finishing on fabrics partially or totally containing aramidic fibre, in the form of filament and/or flock.

As known, aramidic fibres are aromatic polyamides with a content of aromatic groups of more than 85%.

Meta-aramidic fibres are those based upon phenylenediamine-isophthalamide, marketed with the trademark Nomex, the chemical structure of which is shown below.

Normex contains meta-phenylene groups, in other words the amidic groups (NH-CO) are attached to the aromatic ring in positions 1 and 3.

This fibre is suitable for applications where high resistance to heat and flames is required. It has an elastic modulus comparable to that of polyester but less variable with temperature.

These fibres are obtained directly from the polymerisation process since they cannot be melted even at temperatures of over 400°C. Indeed, the polymer deteriorates before melting.

There are also aromatic polyamidic fibres with high mechanical characteristics obtained by humid spinning of a liquid-crystalline solution of p-phenylene diamine and terephthalic chloride polymerized in sulphuric acid: Kevlar.

Kevlar is a para-aramidic fibre, since the aramidic groups are attached in positions 1 and 4, as shown in the figure.

Other fibres classified as meta and para aramidic are known by the trademarks Kennel, Twaron and Conex.

It is also known that so-called "hybrid" fabrics comprise fabrics made with couplings of different types of fibres intended to balance some characteristics or weaknesses of the individual materials.

Frequent examples are those in which aramidic fibres and other fibres of synthetic origin (polyester, polyamide and others) or aramidic fibres and fibres of natural origin (cotton, wool, silk and others) or aramidic fibres and fibres of artificial origin (viscous and others) are woven together.

However, there are many possible types of blends and couplings and they can be made especially for specific conditions of use.

It is also well-known that aramidic fibres display a low surface energy and high chemical inertia, for which reason the adhesion of the printing dyes and of the chemical finishing products, with which they come into contact, is very poor.

Therefore, by applying the printing and finishing processes and techniques currently known to fabrics made with such fibres the end results, in terms of resistance to washing and functional characteristics induced by the finishing, deterioration, appearance and feel, are quite poor.

Normally, the fabrics produced with the aforementioned fibres are nowadays usually printed with pigment-based dyes.

For the above reasons, the fabrics in printed aramidic fibres have low resistance to washing and, moreover, the water-oil repellence values obtained through finishing decrease, often significantly, after the first washes.

The main aesthetic characteristics, such as appearance and feel, after the first washes are greatly altered with respect to the original product, both through the appearance on the surface of parts of fibre not covered by printing or finishing products, and through the substantial loss of printing or finishing products previously applied on the surface.

Moreover, it is very difficult to respect the printing specifications, above all when precise infrared reflectance and/or chromatic tone/intensity values are required.

This drawback becomes of great importance above all in the case of camouflage clothing for military use in which it is vitally important that they have optimal infrared reflectance and chromatic values.

The technical task proposed of the present invention is, therefore, that of making a process for printing and finishing on fabrics partially or totally containing aramidic fibre, in the form of filament and/or flock, which does not have the drawbacks described briefly relative to the prior art.

In this task a purpose of the finding is to make a process for printing and finishing on fabrics partially or totally containing aramidic fibre, in the form of filament and/or flock, which have high resistance to washing and high water-oil repellence values, obtained through finishing, which do not significantly decrease even after numerous washes.

Yet another purpose is to make a process for printing and finishing on fabrics partially or totally containing aramidic fibre, in the form of filament and/or flock, in which the main aesthetic characteristics, such as appearance and feel, after numerous washes, are unchanged with respect to the original product.

A further purpose of the finding is to make a process for printing and finishing on fabrics partially or totally containing aramidic fibre, in the form of filament and/or flock, which does not have the appearance on the surface of parts of fibre not covered by printing or finishing products such as to jeopardise its appearance and that is not subject to the loss of the printing and finishing products previously applied on the surface.

The last but not least purpose is to make a process for printing and finishing on fabrics partially or totally containing aramidic fibre, in the form of filament and/or flock, which respects the specification values, even when precise infrared reflectance and/or chromatic tone/intensity values are required.

This task, as well as these and other purposes are accomplished by a process for printing and finishing on fabrics partially or totally containing aramidic fibre, in the form of filament and/or flock according to claim 1.

Advantageously, the printing process object of the present invention consists of a plasma pre-treatment, a printing process, a process of fixing vat dyes, acid/premetallised dyes, mixture of vat dyes with acid/premetallised dyes, dispersed dyes, cationic dyes or pigment-based dyes, and washing of the fabrics thus treated, in the presence of particular chemical reactants and precise process conditions.

In order to overcome the high chemical inertia of the fabrics made with the fibres described above, unlike the chemical products and the dyes normally used in the field, and in particular, to activate the surface of such fabrics and increase their energy level, a plasma treatment is carried out that, according to requirements, can be carried out only before the printing step or the finishing step or in both cases.

The last situation has given the best results.

According to the present invention, the plasma treatment is preceded by a dehumidification process of the fabric, until a residual humidity level of the fabric is reached that is less than 4% of its weight.

The plasma can be obtained through corona treatment, or through atmospheric plasma or preferably through plasma under vacuum.

In this last case, the plasma can be created by using gas, such as air, oxygen, nitrogen, carbon dioxide, argon, helium, ammonium and various mixtures thereof.

Through the use of such gases plasmas are obtained capable of removing organic contaminants of the surface of the fabric, of increasing the roughness value and of modifying the chemical composition of the surface of the fabric, introducing new chemical groups and free radicals.

The effect of such a surface modification becomes apparent with a significant increase in hydrophily of the fibres making up the fabric, allowing the dyes to spread more uniformly and effectively between the meshes of the fabric and to penetrate more stably in the first molecular layers of the surface of the fibres.

Significant surface modifications of the fabrics in aramidic fibres have been discovered for plasma treatment defined by the following operating intervals:
- gas = oxygen, nitrogen, argon, helium, carbon dioxide, preferably air;
- pressure = 50-180 Pa, preferably 80 Pa
- current intensity = 100-200 A, preferably 180 A, with power supply in the medium frequency field and preferably equal to 10 kHz
- speed = 5-20 m/min, preferably 10 m/min

During the printing preparation step, the fabric is first pre-treated with plasma, impregnated with a suitable swelling agent whose recipe expressed in g/kg could be the following:

| | |
|---|---|
| Water | 798,5 |
| NP Emulsifier | 1,5 |
| Surfadone LP-100 | 200 |

and dried at low temperature.

The printing step is carried out with either flat screen or rotary cylinder processes, making use of vat dyes, or a mixture thereof with pigment-based dyes, cationic dyes, dispersed dyes, 02 acid/premetallised dyes. In particular, the mixture composed of vat dyes and acid/premetallised dyes has given the best results. The printing operation foresees the preparation of the recipe of the printing paste containing the dyes.

In the case of the recipe composed of the mixture of vat dyes with acid/premetallised dyes or dispersed dyes , ingredients are foreseen for giving body to the printing paste, fixing agents and agents which assist in improving the characteristics of the printed fabric.

A composition example of the same is reported below, expressed in g/kg:

| | |
|---|---|
| Water | 746,2 |
| Printex GP 10 | 23 |
| Solvitose C 5 | 23 |
| Preventol P 840 | 0,4 |
| Parmetol | 0,4 |
| Helizarin TW Binder | 100 |
| Resin MFP 98 LF | 15 |
| Neopat compound 96/M | 12 |
| Polyethyleneglycol 300 | 50 |
| Oxiton S/P | 30 |

The vat dyes (or Indanthrene) are added to the printing paste, in mixture with either acid/premetallised dyes or with dispersed dyes, for obtaining the desired tone.

After the step of printing and drying, the latter necessary for evaporating the aqueous part, the following steps sequentially follow:
o vaporising, preferably in a closed chamber at 173°C, 1050 kg/h of superheated vapour for 42' (necessary operation for fixing the acid/premetallised or dispersed dyes)
o developing (necessary operation for fixing the vat dyes ) and stripping the dispersed dyes. These two operations, which can occur simultaneously, are carried out by foulard impregnation (with a squeezing ratio in the range of 50 - 70% of pick-up) of the printed fabric in full bath with the following recipe, expressed in g/kg:

| | |
|---|---|
| Water | 699,8 |
| Granular Borax | 15 |
| Leophen LG | 4 |
| Caustic Soda 48° Bè | 91,2 |
| Potassium Carbonate | 40 |
| Solvitose C5 | 17 |
| Rongalite 2PH-A | 83 |
| Rongalite 2PH-B | 50 |

and vaporising with tower at 168° C, 2700 kg/h superheated vapour flow rate, 90" stay time
o washing in oxidising environment for the presence of hydrogen peroxide at a temperature of 22°C for 2', washing with BIOTEX PS/2 at 98°C for 3', neutralisation with acetic acid at 22°C for 30", final rinse with water at 22°C for 30" and drying with Kenz (ramps) with fabric temperature values of about 80°C.

The water-oil repellent finishes, normally consisting of fluorocarbonic resins, are carried out through impregnation of the fabric in a bath and subsequent drying and polymerisation of the chemical product applied.

The chemical finishing products, as well as giving the desired functionalities to the fabric, in the case of printed fabrics in aramidic fibre according to the present invention carry out a protective action with regard to the printing dyes. Also in this case, the action of the plasma is essential to obtain better results and performance with respect to those that can normally be obtained, since, on the one hand, the chemical finishing product remains anchored to the surface of the treated fabric better and for a longer time, and on the other hand, the higher hydrophily of the fabric ensures a better and complete uniformity of the finishing product on the fibres.

### Example

A 100% Nomex fabric of weight 150 g/m², consisting of 32 strands/cm (count = 45 NM, items = 1), in the form of filament, in warp and 23 strands/cm (count = 101 NM, items = 2), in the form of flock, in weft, was first of all dehumidified, reducing the residual humidity to a value of less than 4% of its weight.

The fabric was then treated with plasma under the following conditions:
- gas = air
- pressure = 80 Pa
- current intensity = 180 A
- speed = 10 m/min,
- equal to an exposition time = 40 sec

The printing of a camouflage design, consisting of the colours maroon, brown, light brown, green and kaki was carried out under the conditions displayed above.

Then the development of the printing was carried out under the conditions displayed above.

Another plasma pre-treatment was carried out before finishing under the following conditions:
- gas = oxygen
- pressure = 80 Pa
- current intensity = 180 A
- speed = 10 m/min,

Finishing was carried out using a standard recipe, suitable for giving water-oil repellence characteristics, through the ordinary application process.

The printing results were measured according to the CIELAB method, through which the chromatographic values of the printed and finished fabric according to the method of the present invention are detected, and they are compared with those obtained through the standard printing process, in other words without plasma preparation, but with the same printing and finishing products.

In particular, for the four colours printed, before washing, the following differences have been noted:
Reference: standard dark brown
Sample: Dark brown (new method)
**DE = 2,971 DL = -0.595DC = -2,911 DH = 0,012**

Reference: standard light brown
Sample: Light brown (new method)
**DE = 1,715 DL = -1,261DC = -1,162 DH = 0,007**

Reference: standard green
Sample: Green (new method)
**DE = 1,788 DL = -0,771DC = -1,605 DH = 0,164**

Reference: standard kaki
Sample: Kaki (new method)
**DE = 1,386 DL = -0,033DC = -1,385 DH = 0,035**

These values demonstrate that, for all four of the colours printed, there are total colour differences **DE**, which are more or less pronounced according to whether the colour is light or dark.

In particular, the negative value of **DL** (difference in lightness) indicates the darker value of the colour obtained on fabrics printed according to the present invention, the negative value of **DC** (difference in chromaticity) indicates the lower saturation value of the colour obtained on the fabrics printed according to the present invention, the almost unchanged value of **DH** (difference in hue) indicates that the total difference in colour obtained with the application of the two methods does not depend upon a difference in hue, since there is not one, but mainly upon the colour saturation and upon the lightness, for the darker colours.

Then the end characteristics of the standard product and the product made according to the present invention were measured and compared, the results of which are displayed in the following table:

| OLEOPHOBOL 7752 | g/l | \ | Drying 1' at 110°C - polymerisation 3' at 160°C |
|---|---|---|---|
| NUVA HP | g/l | 80 | PK recipe 2: 51.5 % |
| ACETIC ACID | g/l | 1 | |
| HYDROPHOBOL XAN | g/l | \ | |
| FLEXANOL SOLVENT | g/l | 10 | |

| | | | | Standard sample | Plasma treated sample |
|---|---|---|---|---|---|
| **PHYSICAL PERFORMANCE** | | | | | |
| **OIL REPELLENCY** STANDARD AATCC118 | | As such | | 6 | 6 |
| | | After 5 washes at 60°C# | not ironed | 4 | 4 |
| | | After 5 washes at 60°C# | ironed | 5 | 5 |
| **SPRAY TEST** STANDARD AATCC22 | | As such | | 100 | 100 |
| | | After 5 washes at 60°C# | not ironed | 100 | 100 |
| | | | | | |
| **SOLIDITY OF COLOURS** | | | | | |
| **RUBBING** STANDARD EN ISO 105 X12 | | dry | | 3 | 3 |
| | | wet | | 3/4 | 3/4 |
| **DETERIORATION OF COLOUR AFTER 5 WASHES AT 60°C#** #EN ISO 6330 2AE | | | Brown | 2 | 4 |
| | | | Light brown | 3 | 4 |
| | | | Kaki | 4 | 4/5 |
| | | | Green | 4 | 4/5 |

| | | | | | |
|---|---|---|---|---|---|
| * Air 10' 80 Pa 180 A Polymerisation : Arioli 173°C x 10' x 1000 kg/h steam - Two steps scheme 1 recipe 2 speed 25 ** Oxygen 10' 80 Pa 180 A | | | | | |

Although there are no differences in terms of physical performance between the two samples, there are significant differences in the results with regard to the deterioration of the colours after washing, which make the sample obtained with the new method in accordance with the values required (3/4) in various fields of application in which its use is currently prevented due to the fact that the minimum solidity requirements have not been met.

In practice, it has been noted how the process for printing and finishing on fabrics partially or totally containing aramidic fibre according to the present invention is particularly advantageous to be able to offer increased resistance to washing of the printing dyes and of the chemical finishing products, conserving technical and aesthetic characteristics much more similar to the original product compared to what can be obtained with known techniques.

## Claims

1. Process for printing and finishing on fabrics partially or totally containing aramidic fibre, in the form of filament and/or flock, **characterised in that** it consists of carrying out a plasma treatment on the fabric only before the printing process and/or before the finishing process, wherein before the plasma treatments a dehumidification process of the fabric is carried out until a residual humidity level of the fabric of less than 4% of its weight and preferably less than 3% is reached,

2. Printing and finishing process according to one or more of the previous claims, **characterised in that** said plasma treatment is carried out through plasma in a vacuum.

3. Printing and finishing process according to claim 1 , **characterised in that** said plasma treatment is carried out through atmospheric plasma.

4. Printing and finishing process according to one or more of the previous claims, **characterised in that** said plasma treatment is carried out through corona treatment.

5. Printing and finishing process according to claim 2 , **characterised in that** said vacuum plasma treatment is carried out through a plasma created using gas and preferably air, oxygen, nitrogen, carbon dioxide, argon, helium or ammonia or various mixtures of these and **characterized by** using vat dyes or a mixture of vat dyes and
pigment-based dyes, cationic dyes, dispersed dyes or acid/premetallised dyes for carrying out the printing. gases.

6. Printing and finishing process according to claims 2 or 5 , **characterised in that** the operating pressure of said plasma is between 50 and 180 Pa and preferably it is 80 Pa.

7. Printing and finishing process according to one or more of the previous claims, **characterised in that** the current intensity of said plasma is between 100 and 200 A and preferably it is 180 A, with power supply in the medium frequency field and preferably equal to 10 kHz.

8. Printing and finishing process according to one or more of the previous claims, **characterised in that** the speed of said plasma is between 5 and 20 m/min and preferably it is 10m/min.

9. Printing and finishing process according to one or more of the previous claims, **characterised in that** said finishing process is of the water-oil repellent type, consisting of fluorocarbonic resins and carried out through impregnation of the fabric in a bath and subsequent drying and polymerisation of the chemical product applied.

10. Printing and finishing process according to one or more of the previous claims, **characterised in that** during the printing preparation step, the fabric is first pre-treated with plasma, then impregnated with a suitable swelling agent, and then dried at low temperature.

11. Printing and finishing process according to one or more of the previous claims, **characterised in that** in the case of a dyes recipe composed of the mixture of vat dyes with acid/premetallised dyes or dispersed dyes or composed only of acid/premetallised dyes, ingredients are foreseen for giving body to the printing paste, fixing agents and agents which assist in improving the characteristics of the printed fabric.

12. Printing and finishing process according to one or more of the previous claims, **characterised in that** after the step of printing and drying, the latter necessary for evaporating the aqueous part, follow the steps of vaporising, necessary for fixing the acid/premetallised or dispersed dyes, if they are present in said recipe; and/or developing, necessary for fixing the vat dyes if they are present in said recipe.

13. Fabric partially or totally containing aramidic fibre, in the form of filament and/or flock, **characterised in that** it has been treated according to the process claimed in one or more of the previous claims.

## Patentansprüche

1. Verfahren zum Bedrucken und zur Oberflächenbehandlung von Geweben, die teilweise oder vollständig aramide Fasern in Form von Filamenten und/oder Kurzfasern enthalten, **dadurch gekennzeichnet, dass** es aus der Ausführung einer Plasmabehandlung des Gewebes erst vor dem Druckverfahren und/oder vor dem Oberflächenbehandlungsverfahren besteht, wobei vor der Plasmabehandlung ein Entfeuchtungsverfahren des Gewebes ausgeführt wird, bis ein Restfeuchtigkeitsgrad des Gewebes von weniger als 4 % seines Gewichts und vorzugsweise weniger als 3 % erreicht wird, und **dadurch gekennzeichnet, dass** Küpenfarbstoffe oder eine Mischung aus Küpenfarbstoffen und pigmentbasierten Farbstoffen, kationischen Farbstoffen, dispergierten Farbstoffen oder Säure-/vormetallisierten Farbstoffen zur Ausführung des Drucks verwendet werden.

2. Bedruckungs- und Oberflächenbehandlungsverfahren nach einem oder mehreren der vorangehenden Ansprüche, **dadurch gekennzeichnet, dass** die Plasmabehandlung durch Plasma in einem Vakuum ausgeführt wird.

3. Bedruckungs- und Oberflächenbehandlungsverfahren nach Anspruch 1, **dadurch gekennzeichnet, dass** die Plasmabehandlung durch atmosphärisches Plasma ausgeführt wird.

4. Bedruckungs- und Oberflächenbehandlungsverfahren nach einem oder mehreren der vorangehenden Ansprüche, **dadurch gekennzeichnet, dass** die Plasmabehandlung durch Koronabehandlung ausgeführt wird.

5. Bedruckungs- und Oberflächenbehandlungsverfahren nach Anspruch 2, **dadurch gekennzeichnet, dass** die Vakuumplasmabehandlung durch ein Plasma ausgeführt wird, das durch die Verwendung von Gas und vorzugsweise Luft, Sauerstoff, Stickstoff, Kohlendioxid, Argon, Helium oder Ammoniak oder unterschiedlichen Mischungen dieser Gase erzeugt wird.

6. Bedruckungs- und Oberflächenbehandlungsverfahren nach den Ansprüchen 2 oder 5, **dadurch gekennzeichnet, dass** der Betriebsdruck des Plasmas zwischen 50 und 180 Pa liegt und vorzugsweise 80 Pa beträgt.

7. Bedruckungs- und Oberflächenbehandlungsverfahren nach einem oder mehreren der vorangehenden Ansprüche, **dadurch gekennzeichnet, dass** die Stromdichte des Plasmas zwischen 100 und 200 A liegt und vorzugsweise 180 A beträgt, mit einer Stromversorgung im Mittelfrequenzfeld und vorzugsweise gleich 10 kHz.

8. Bedruckungs- und Oberflächenbehandlungsverfahren nach einem oder mehreren der vorangehenden Ansprüche, **dadurch gekennzeichnet, dass** die Geschwindigkeit des Plasmas zwischen 5 und 20 m/min liegt und vorzugsweise 10 m/min beträgt.

9. Bedruckungs- und Oberflächenbehandlungsverfahren nach einem oder mehreren der vorangehenden Ansprüche, **dadurch gekennzeichnet, dass** das Oberflächenbehandlungsverfahren vom Wasser-Öl-abweisenden Typ ist, bestehend aus Fluorcarbonharzen und ausgeführt durch die Imprägnierung des Gewebes in einem Bad und anschließendes Trocknen und Polymerisieren des aufgetragenen chemischen Produkts.

10. Bedruckungs- und Oberflächenbehandlungsverfahren nach einem oder mehreren der vorangehenden Ansprüche, **dadurch gekennzeichnet, dass** das Gewebe während des Bedruckungsvorbereitungsschrittes zuerst mit Plasma vorbehandelt, anschließend mit einem geeigneten Quellungsmittel imprägniert und danach bei niedrigen Temperaturen getrocknet wird.

11. Bedruckungs- und Oberflächenbehandlungsverfahren nach einem oder mehreren der vorangehenden Ansprüche, **dadurch gekennzeichnet, dass** im Falle eines Farbstoffrezepts, sich zusammensetzend aus der Mischung von Küpenfarbstoffen mit Säure-/vormetallisierten Farbstoffen oder dispergierten Farbstoffen oder sich nur aus Säure-/vormetallisierten Farbstoffen zusammensetzend, Zutaten, die der Druckpaste Substanz verleihen, Fixiermittel und Mittel, die bei der Verbesserung der Eigenschaften des bedruckten Gewebes helfen, vorgesehen sind.

12. Bedruckungs- und Oberflächenbehandlungsverfahren nach einem oder mehreren der vorangehenden Ansprüche, **dadurch gekennzeichnet, dass** nach dem Schritt des Bedruckens und Trocknens, wobei Letzterer zum Verdampfen des wässrigen Teils notwendig ist, die Schritte des Verdampfens, notwendig zum Fixieren der Säure-/vormetallisierten oder dispergierten Farbstoffe, wenn sie im Rezept vorhanden sind, und/oder des Entwickelns, notwendig zum Fixieren der Küpenfarbstoffe, wenn sie im Rezept vorhanden sind, folgen.

13. Gewebe, das vollständig oder teilweise aramide Fasern in Form von Filamenten und/oder Kurzfasern enthält, **dadurch gekennzeichnet, dass** es gemäß dem Verfahren nach einem oder mehreren der vorangehenden Ansprüche behandelt wurde.

## Revendications

1. Procédé d'impression et de finition de tissus étant constitués en partie ou en totalité de fibres aramides, sous forme de filaments et/ou de flocs, **caractérisé en ce qu'**il consiste à effectuer un traitement plasma sur le tissu uniquement avant le procédé d'impression et/ou avant le procédé de finition, dans lequel est mené un procédé de déshumidification du tissu avant le traitement plasma jusqu'à atteindre un taux d'humidité résiduelle du tissu égal à moins de 4% de son poids, et de préférence à moins de 3%, et **caractérisé en ce qu'**il utilise des colorants de cuve ou un mélange de colorants de cuves et de colorants à base de pigments, des colorants cationiques, des colorants plastosolubles ou des colorants acides/prémétallisés pour faire l'impression.

2. Procédé d'impression et de finition selon une ou plusieurs des revendications précédentes, **caractérisé en ce que** ledit traitement plasma est mené par plasma sous vide.

3. Procédé d'impression et de finition selon la revendication 1, **caractérisé en ce que** ledit traitement plasma est mené par plasma atmosphérique.

4. Procédé d'impression et de finition selon une ou plusieurs des revendications précédentes, **caractérisé en ce que** ledit traitement plasma est mené par décharge couronne.

5. Procédé d'impression et de finition selon la revendication 2, **caractérisé en ce que** ledit traitement par plasma sous vide est mené par un plasma généré avec un gaz, et de préférence, l'air, l'oxygène, l'azote, le dioxyde de carbone, l'argon, l'hélium ou l'ammoniac ou divers mélanges de ces gaz.

6. Procédé d'impression et de finition selon les revendications 2 ou 5, **caractérisé en ce que** la pression de travail dudit plasma se situe entre 50 et 180 Pa, et de préférence est de 80 Pa.

7. Procédé d'impression et de finition selon une ou plusieurs des revendications précédentes, **caractérisé en ce que** l'intensité de courant dudit plasma se situe entre 100 et 200 A, et de préférence est de 180 A, avec alimentation à moyenne fréquence, et de préférence égale à 10 kHz.

8. Procédé d'impression et de finition selon une ou plusieurs des revendications précédentes, **caractérisé en ce que** la vitesse dudit plasma se situe entre 5 et 20 m/min, et de préférence est de 10 m/min.

9. Procédé d'impression et de finition selon une ou plusieurs des revendications précédentes, **caractérisé en ce que** ledit procédé de finition est du type hydrophobe/oléophobe, consistant en des résines fluorocarbonées, et est mené par imprégnation du tissu dans un bain, puis par séchage et par polymérisation du produit chimique appliqué.

10. Procédé d'impression et de finition selon une ou plusieurs des revendications précédentes, **caractérisé en ce que**, pendant l'étape de préparation de l'impression, le tissu est d'abord prétraité par plasma, puis imprégné d'un agent de gonflement approprié, et ensuite séché à basse température.

11. Procédé d'impression et de finition selon une ou plusieurs des revendications précédentes, **caractérisé en ce que**, dans le cas d'une formule de colorants composée du mélange de colorants de cuves et de colorants acides/prémétallisés ou de colorants plastosolubles ou composée uniquement de colorants acides/prémétallisés, il est prévu des ingrédients pour donner de la consistance à la pâte d'impression, des agents de fixation et des agents qui contribuent à améliorer les caractéristiques du tissu imprimé.

12. Procédé d'impression et de finition selon une ou plusieurs des revendications précédentes, **caractérisé en ce que**, après l'étape d'impression et l'étape de séchage, cette dernière nécessaire pour faire évaporer la partie aqueuse, il s'ensuit l'étape de vaporisation, nécessaire pour fixer les colorants acides/prémétallisés ou les colorants plastosolubles, s'ils sont présents dans ladite formule ; et/ou l'étape de développement, nécessaire pour fixer les colorants de cuve, s'ils sont présents dans ladite formule.

13. Tissu étant constitué en partie ou en totalité de fibres aramides, sous forme de filaments et/ou de flocs, **caractérisé en ce qu'**il a été traité selon le procédé décrit dans une ou plusieurs des revendications précédentes.
